

No. 717,793.

PATENTED JAN. 6, 1903.

L. M. J. ARMANDY.

MANUFACTURE OF PHOTOGRAPHIC FILMS.

APPLICATION FILED DEC. 2, 1901.

NO MODEL.

Fig. 1.



Fig. 2.



Fig. 3.



WITNESSES :

*W. M. Avery*

*H. H. Bernhardt*

INVENTOR

*Leon M. J. Armandy*

BY

*Wm. S.*

ATTORNEYS

# UNITED STATES PATENT OFFICE.

LÉON MARIE JOSEPH ARMANDY, OF ASNIÈRES, FRANCE, ASSIGNOR TO  
SOCIÉTÉ ANONYME DES PRODUITS PHOTOGRAPHIQUES M. Y. OF AS-  
NIÈRES, SEINE, FRANCE.

## MANUFACTURE OF PHOTOGRAPHIC FILMS.

SPECIFICATION forming part of Letters Patent No. 717,793, dated January 6, 1903.

Application filed December 2, 1901. Serial No. 84,365. (No specimens.)

*To all whom it may concern:*

Be it known that I, LÉON MARIE JOSEPH ARMANDY, engineer, a citizen of the Republic of France, and a resident of 3 Rue Brantôme, Asnières, Seine, Republic of France, have invented Improvements Relating to the Manufacture of Photographic Films, of which the following is a full, clear, and exact description.

10 This invention relates to the manufacture of films for photographic purposes, and has for its object to provide improved means whereby such films may be readily detached from their support or backing.

15 My invention consists, essentially, in arranging between the support or backing and the sensitized film a layer of suitable material capable of imparting to the film a certain plasticity and of being readily dissolved out 20 during the ordinary operations of developing, fixing, and washing.

I have found that a layer of gelatin spread upon a backing or support of paper or the like previously coated with an appropriate 25 solution of gum or resin will readily detach itself after drying, without any necessity of applying a solvent for the said gum or resin. I also have found that by adding to the gelatin a substance for softening it the latter remains 30 adherent to the backing or support by reason of the suppleness imparted to it, the separation being effected when the said substance has been eliminated by the various photographic baths—*i. e.*, when the gelatin has returned to its original condition.

35 My improved process comprises the following operations: I first coat the backing or support, of paper or the like, with a solution of dammar-gum in benzene, and after the 40 evaporation of the solvent I spread upon said backing or support a solution of gelatin which may contain, according to the purposes to which it is to be applied, alum, tannin, &c., with an addition of glycerin or another similar substance. The “similar substance” just referred to may consist of sugar, honey, or gum; but these ingredients are not, properly speaking, the equivalents of the glycerin. The addition of said ingredients to the glycerin and the gelatin film produces similar ef-

fects—that is, the incorporation of the sugar, honey, and gum or a mixture of them into the gelatin serves to give the necessary plasticity to the gelatin, and such admixture causes the gelatinous coating or film to adhere to the support or backing which is supplied with the resinous coating heretofore described. These divers products are eliminated by the different baths to which the photographic film is subjected during development, &c., and the elimination of the adhesive agents serves to permit the gelatin film to again assume after desiccation its natural rigidity and to detach itself spontaneously from the backing or support. This 60 produces a perfect adherence between the backing or support and the gelatin even after complete drying, and the product thus obtained can be readily preserved without experiencing any alteration, provided it is kept 65 dry. The material may be folded, rolled, receives other layers—for example, sensitive photographic coatings—without separation taking place and without losing any of its suppleness. When the product thus obtained 70 is subjected to the various photographic baths, the glycerin or similar product which has been incorporated in the gelatin is eliminated from the latter, and after drying the said gelatin, which then has returned to its 75 original condition, constitutes a stiff sheet and spontaneously abandons the backing or support.

According to the different results it is desired to obtain, my process may comprise also 85 the following operations: When coating a backing or support of paper or the like with a covering of gelatin, whether or not it has first been coated with gum or resin, the gelatin in drying reproduces exactly the grain of 90 the paper or the like, and the film used as a positive or negative for printing again reproduces it. In order to avoid this objection, I apply to the backing or support a preliminary coating of gum-lac dissolved either in a solution of borax or in a solution of sodium carbonate, ammonium carbonate, or other similar alkaline substance. This first dressing prevents the grain of the backing or support 95 being reproduced in the subsequent coatings. 100

The gelatin coating, however perfect it may be, presents irregularities which prejudice the appearance of the photographic picture obtained by means of this negative printing-  
 5 film or of the positive transparent picture, and therefore necessitates the use of a paper or matted glass for a backing or lining. I am enabled to avoid the said objection by de-  
 10 polishing the gelatin coating. For this pur-  
 pose I add to the gelatin either starch, arrow-  
 root, or any fecula or the precipitate of ba-  
 15 rium sulfate produced in the mass or, better, added after the complete purification by wash-  
 ing. This addition may be made either in  
 20 the gelatin only or also in the superposed  
 sensitive coating or film. Lastly, I obtain  
 superior results in forming coatings upon the  
 25 backing or support—*i. e.*, by covering the lat-  
 ter with a preliminary gelatin layer, to which  
 is added barium sulfate strongly alumed—  
 and glazing in a calendering-roller the said  
 30 preliminary coating. According to my mode  
 of manufacture the successive coatings are ap-  
 plied either with a brush or by dipping or  
 35 mechanically by means of a machine and ac-  
 cording to the methods used in the manufac-  
 ture of coated papers or photographic papers.

In the drawings herein annexed, Figure 1  
 30 is a perspective view of my stripping photo-  
 graphic film. Fig. 2 is a like view of back-  
 ing after separation thereof from the gelatin  
 film, and Fig. 3 is a like view of the gelatin  
 film.

A designates the pliable backing, which  
 35 may be of paper, tissue, or any other suitable  
 material to form the support. On this back-  
 ing or support is adapted to be spread a layer  
 of gum-lac varnish, (indicated at B,) and over  
 40 said layer B is applied the coating C, having  
 a resinous base.

D designates the gelatin film, and E is the  
 45 sensitized coating thereon.

The photographic film may be exposed and  
 developed in the usual way, and after the op-  
 eration is completed the film separates into  
 45 two distinct parts, one of which is shown by  
 Fig. 2 and the other by Fig. 3. One part con-

sists of the paper support, the varnish layer,  
 and the resinous coating, while the other part  
 is composed of the gelatin film having the sen-  
 50 sitized surface.

I claim—

1. An improved process of manufacturing  
 photographic films, which consists in spread-  
 ing upon a backing a stripping layer com-  
 55 posed of a gummy solution, spreading upon  
 said stripping layer a layer of gelatin mixed  
 with an adhesive soluble substance which im-  
 parts the required suppleness thereto, and  
 60 spreading upon said gelatin layer a sensitized  
 film.

2. A process of making photographic films,  
 which consists in spreading upon a backing  
 a stripping layer composed of a gummy solu-  
 65 tion, spreading upon said stripping layer a  
 layer of gelatin mixed with an adhesive solu-  
 ble substance, subjecting the gelatin coating  
 to the action of a depolishing agent, and  
 70 spreading upon the gelatin layer a sensitized  
 film.

3. A process of making photographic films,  
 which consists in producing a polished sur-  
 face on a backing, spreading thereon a layer  
 of gelatin mixed with an adhesive soluble  
 75 substance which imparts the required supple-  
 ness thereto, and applying upon said gelatin  
 layer a sensitized film.

4. A process of making photographic films,  
 which consists in producing a polished sur-  
 face on a suitable backing by applying there-  
 80 to a coating of gum-lac varnish; applying a  
 resinous coating; spreading on said resinous  
 coating a layer of gelatin mixed with an ad-  
 hesive soluble substance which imparts the  
 85 required suppleness thereto, and spreading  
 upon said gelatin layer a sensitized film.

The foregoing specification of my improve-  
 ments relating to the manufacture of photo-  
 graphic films signed by me this 19th day of  
 November, 1901.

LÉON MARIE JOSEPH ARMANDY.

Witnesses:

EDWARD P. MACLEAN,  
 MAURICE H. PIGNET.